# EUROPEAN PATENT SPECIFICATION

(11) **EP 0 275 844 B1**
(45) Date of publication and mention of the grant of the patent: **28.07.1993**
(21) Application number: 87830452.6
(22) Date of filing: 21.12.1987
(51) Int. Cl.: H01J 7/18

(54) **Non evaporable getter device incorporating a ceramic support and method for the manufacture thereof**
Mit einem keramischen Träger versehene, nicht verdampfbare Gettervorrichtung und Herstellungsverfahren derselben
Dispositif getter non évaporable comportant un support céramique et son procédé de fabrication

(30) Priority: 22.12.1986 IT 2280786
(43) Date of publication of application: 27.07.1988
(73) Proprietor: SAES GETTERS S.P.A., I-20151 Milano (IT)
(72) Inventor: Boffito, Claudio, I-20017 Rho (Milano) (IT); Giorgi, Ettore, Milano 2 I-20090 Segrate (Milano) (IT)
(74) Representative: Adorno, Silvano

(56) References cited:
- FR-A- 2 447 745
- GB-A- 2 000 370
- GB-A- 2 157 073
- US-A- 3 620 645

## Description

The present invention relates to a non-evaporable getter device comprising a ceramic support, as well as a method for the manufacture of such a device.

Non-evaporable getter devices are well-known in the art. They usually consist of a powdered metal or alloy which when heated to an elevated temperature, diffuse into the bulk a protective layer such that the surface of the particles become reactive towards a large number of gases.

In this active conditions they are capable of producing or maintaining a high vacuum.

Usually the non-evaporable getter material is held in a support such as, for instance, by pressing the powder into a U-shaped metal ring channel.

Another type of support has been described in US Patent US-A-3,620,645 in which the getter material is pressure bonded onto the surface of a continuous metal strip. UK Patent Application GB-A-2,157,486 describes the electrophoretic deposition of getter material onto a wide variety of supports.

One particular embodiment briefly described is a wire which has previously been coated with a ceramic insulating material such as alumina. The wire coated with alumina is used as one electrode in an electrophoretic coating bath in which there are suspended particles of the getter material. The getter material is electrophoretically deposited onto the ceramic coated wire. Unfortunately the use of such a support has several disadvantages. Firstly the alumina layer on the wire must be very thin otherwise it is very difficult to cause sufficient electric current to flow to effect the deposition. Due to the high electrical resistance of the alumina coating it is also very difficult to control the parameters of deposition, resulting in an uneven deposition. An additional difficulty is that during a subsequent sintering process the electrophoretically deposited getter material detaches from the ceramic support producing flakes and undesirable loose particles.

It is an object of the present invention to provide a porous non-evaporable getter device having a ceramic support in which during and after a sintering process the getter material remains firmly attached to the support.

It is another object of the present invention to provide a method for the manufacture of a porous non-evaporable getter device having a ceramic support in which it is possible to accurately control the electrophoretic deposition characteristics.

These objects are achieved by a getter device showing the features of claim 1 and particularly of the relevant sub-claims 2-7, as well as through a method according to claim 8 and possibly relevant dependent claims 9-10.

Additional objects, advantages and characteristics of the present invention and its method of manufacture will become evident to those skilled in the art by reference to a preferred embodiment described as a non-limiting example with reference to the attached drawings in which:
FIGURE 1 is a diagramatic representation of a getter device of the present invention before being subjected to a sintering process;
FIGURE 2 is a diagramatic representation of a porous non-evaporable getter device of the present invention after being subjected to a sintering process;
FIGURE 3 is a cross-section of a prior art getter device showing detachment of porous non-evaporable getter material from a ceramic support; and
FIGURE 4 is a cross-section of a porous non-evaporable getter device of the present invention showing good adhesion of the non-evaporable getter material to the ceramic support.

It has surprisingly been found that if a metallic layer is provided between the ceramic support and the electrophoretically deposited non-evaporable getter material not only is it possible to accurately control the deposition characteristics of the getter material, but also after the sintering process the porous non-evaporable getter material is firmly held in contact with the ceramic support without any detachment.

In order to manufacture a porous non-evaporable getter device of the present invention, a ceramic support is coated with a thin electrically conductive film. The ceramic support may be of any ceramic material which is compatible with use in high vacuum, preferably alumina. It may be of any shape size or thickness. The thin conductive film may be of any conductive material such as tin oxide or other conductive oxides. It is preferable however to use a thin metal layer such as aluminium or copper. The ceramic may be coated with this thin metallic film by any known method such as electroplating or by deposition in vacuum. The thin metal film can be Ni, Cu, Ag, Mo or Fe but is preferably aluminium. Its thickness is preferably between 0.1 µm and 5 µm. The thin conductive film is then made to be one electrode of an electroplating bath. Upon this thin (preferably aluminium) film there is electroplated a thicker metallic film having a thickness of several micrometers and preferably between 5 µm and 50 µm. The electroplated metal film may be of any metal which is compatible with use in high vacuum such as Ti, Zr, Mo, Fe, Cu, Ag, Pt, Au but it is preferably nickel.

The thin conductive film and the thicker metal layer constitute an intermediate electrically conductive layer which could however be a single metallic layer.

The electroplated support is electrophoretically coated with a mixture of a particulate non-evaporable getter material and an antisintering material. The electrophoretic coating takes place according to a process as described in UK Patent application publication GB-A-2,157,486.

The particular non-evaporable getter material is any getter material suitable for the sorption of active gases in vacuum. It is preferably chosen from the group consisting of titanium, zirconium and their hydrides. Its particle size should be between 20-60 µm and preferably with an average size of 40 µm.

The antisintering material is in particulate form and is any material which is capable of hindering the sintering of the non-evaporable getter material. It is preferably chosen from the group consisting of graphite, refractory metals and metallic getter alloys (particularly zirconium based alloys). If a zirconium based alloy is used as an antisintering material, then it is preferably chosen from the group consisting of:
A. an alloy of zirconium with aluminium in which the weight percent of aluminium is from 5-30%;
B. an alloy of zirconium with M₁ and M₂ where M₁ is chosen from the group consisting of vanadium or niobium and M₂ is chosen from the group consisting of iron or nickel;
C. an alloy of Zr-V-Fe whose composition in weight percent, when plotted on a ternary composition diagram in weight percent Zr, weight percent V and weight percent Fe, lies within a polygon having as its corners the points defined by:
   i) 75% Zr - 20% V - 5% Fe
   ii) 45% Zr - 20% V - 35% Fe
   iii) 45% Zr - 50% V - 5% Fe

Particularly advantageous is the use of an alloy containing 70% Zr, 24.6% V, and 5.4% Fe.

The antisintering material preferably has a particle size of between 20-60 µm with an average particle size of 40 µ. The weight ratio of the particulate non-evaporable getter material to the particulate antisintering material is from 1 : 4 to 4 : 1. After the electroplated ceramic support has been electrophoretically coated to the desired thickness of porous non-evaporable getter material is then removed from the coating bath and rinsed with a suitable liquid such as acetone and then it is dried. It is then heated in vacuum oven at a pressure preferably less than 10⁻⁵Torr (10⁻³ Pa) at a temperature of between about 350°C and 450°C. If a hydrided material is used as the getter material then this temperature should be maintained for a sufficient time as to release all hydrogen. The getter device is then heated at a higher temperature such as between 900°C and 1000°C to produce a porous non-evaporable getter device in which the thicker metal layer diffuses into the ceramic support and the electrophoretically coated getter mixture. The getter device is then allowed to cool to room teperature whereupon it is removed from the vacuum oven and is ready for use.

The term "sintering" as used herein refers to the process of heating powdered material at a temperature and for a time sufficient to give some mass transfer between adjacent particles without appreciably reducing the surface area of the powdered material. The mass transfer serves to bind the particles together thereby increasing strength and reducing the number of loose particles. Lower temperatures require longer times. The sintering temperature of a material is that temperature at which the above-described sintering takes place in about one hour. In a preferred embodiment of the present invention a temperature is chosen which is at or slightly above the sintering temperature of the non-evaporable getter material and below the sintering temperature of the antisintering material.

As it is used herein the term "ceramic" means any material that is not electrically conductive at the temperature of use including glass-ceramics, quartz-glass, SiO₂, refractory metal oxides in general and Al₂O₃ in particular.

Figure 1 shows a porous non-evaporable getter device 102 comprising a ceramic substrate 104. Ceramic support 104 has one of its surfaces 106 coated with a thin film 108 of conductive material. On the thin film 108 of conductive material is an electrodeposited thicker layer 110 of metal. Onto thicker film 110 has been electrophoretically deposited particles 112, 112' of particulate non-evaporable getter material and particles 114, 114' of antisintering material.

Figure 2 shows a porous non-evaporable getter device 202 similar to that shown in Fig. 1 except that it has now been subject to a sintering process. Getter device 202 comprises a ceramic support 204 that supports particles of non-evaporable getter material 206, 206' and particles 208, 208' of antisintering material. As a result of the sintering process the thin and thick conductive layers have diffused into the ceramic to produce a diffusion layer 210 and they have diffused into the getter and/or antisintering material particles to produce diffusion zones 212, 212'. As mentioned above these diffusion zones may result from a single metallic layer.

### EXAMPLE 1

This comparative example was designed to show the behaviour of a prior art porous non-evaporable getter device comprising a ceramic support and a porous sintered getter material layer. A metallic wire was coated with a thin layer of alumina thereby forming a tube which was coated electrophoretically following the process as described in the above mentioned UK Patent Application Publication GB-A-2,157,486 using getter material particles of titanium hydride and antisintering particles of a Zr-V-Fe alloy both having a particle size of approximately 40 µm. After the sintering process and cooling down to room temperature a metallurgical cross-section was made and is shown in Fig. 3.

In order to start the electrophoretic process it was necessary to apply a voltage of 50 V. To maintain a current flow of 800 milliamps it was necessary to rapidly increase the voltage over a period of about 5 seconds. At this time the formation of H₂ gas had commenced making the deposited getter layer have a very rough irregular appearance with spots having no getter metal at all. The deposition of getter material is insufficient. The getter material exhibits undesirable flaking, and produces a large quantity of undesirable loose particles.

Figure 3 shows the cross-section 302 where can be seen the ceramic support 304 of alumina. The sintered non-evaporable getter material 306 comprising titanium and Zr-V-Fe is found to be separated from the ceramic support 304 by a space 308 showing a detachment of the getter material 306 from the ceramic support 304.

### EXAMPLE 2

This example is designed to show the behaviour of a porous non-evaporable getter device of the present invention. An alumina tube was taken and its external surface was coated with aluminium in a vacuum deposition apparatus. Using the aluminium film as an electrode a thicker layer of Ni was electroplated upon it. The Ni layer was then used as an electrode in an electrophoretic deposition bath exactly as for Example 1. The porous non-evaporable getter material again comprised Ti hydride and a Zr-V-Fe alloy as an antisintering agent. The particle size of both components was approximately 40 µm. After the sintering operation and cooling to room temperature a cross-section 402 of the getter device was made and reported in Fig. 4. The alumina support 404 and the getter material 406 are shown to be clearly adhering to each other along line 408. The aluminium and nickel layers can no longer be seen as they have diffused into the alumina and the getter material.

In this case the deposition took place in a few seconds at an applied voltage of 15 V with the passage of 1 ampere. No H₂ formation was observed and the deposition was able to take place for 20 seconds thus providing a sufficient quantity of getter material with a smooth uniform surface appearance.

### EXAMPLE 3

This example illustrates that embodiment of the present invention wherein the intermediate electrically conductive layer is a single metal.

The procedure of Example 2 is repeated except that the aluminium is replaced with nickel such that the intermediate electrically conductive layer is substantially all nickel.

Although the invention has been described in detail with reference to certain preferred embodiments and applications it is intended that variations and modifications can be made within the scope of the claims.

## Claims

1. A porous non-evaporable getter device (102; 202) comprising:
I. a ceramic support (104; 204);
II. a porous sintered getter material layer comprising:
A. a particulate non-evaporable getter material (112,112'; 206,206') and
B. a particulate antisintering material (114,114'; 208,208'), characterized by further comprising:
III. an intermediate electrically conductive layer (108, 110) at least partially diffused (210; 212,212') into che ceramic support and the porous sintered getter material layer.

2. A getter device according to claim 1, characterized in that the ceramic support (104; 204) is alumina.

3. A getter device according to claim 1, characterized in that the particulate non-evaporable getter material (112,112'; 206,206') is chosen from the group consisting of titanium, zirconium and their hydrides.

4. A getter device according to claim 1, characterized in that the particulate antisintering material (114,114'; 208, 208') is chosen from the group consisting of graphite, refractory metals and metallic getter alloys.

5. A getter device according to claim 4, characterized in that the antisintering material is a zirconium based alloy.

6. A porous non-evaporable getter device (102; 202) according to claims 2-5, characterized in that said intermediate electrically conductive layer comprises:
A. a thin film (108) of aluminium; and
B. A thicker layer (110) of nickel at least partially diffused into the alumina support (104; 204) and the porous sintered getter material layer.

7. A getter device according to claim 6, characterized in that the zirconium based alloy is chosen from the group consisting of:
A. an alloy of zirconium with aluminium in which the weight percent of aluminium is 5-30%;
B. an alloy of zirconium with metals M₁ and M₂, wherein M₁ is chosen from the group consisting of vanadium and niobium and M₂ is chosen from the group comprising iron and nickel;and
C. an alloy of Zr-V-Fe whose composition in weight percent, when plotted on a ternary composition diagram in weight percent Zr, weight percent V and weight percent Fe, lies within a polygon having as its corners the points defined by:
i) 75% Zr - 20% V - 5% Fe
ii) 45% Zr - 20% V -35% Fe
iii) 45% Zr - 50% V- 5% Fe

8. A method for manufacturing a porous non-evaporable getter device, characterized by comprising the steps of:
I. coating a ceramic support (104; 204) with a thin conductive film (108);
II. electroplating the thin conductive film (108) with a thicker metal layer (110) to produce an electroplated support;
III. electrophoretically coating the electroplated support with a mixture of:
A. a particulate non-evaporable getter material (112,112'; 206,206'); and
B. a particulate antisintering material (114,114'; 208,208') to produce a coated support;
IV. sintering the coated support at super-ambient temperatures to produce the porous, non-evaporable getter device; whereby the electroplated thicker metal layer (110) diffuses into the ceramic support (104; 204) and the electrophoretically coated mixture; and then
V. cooling said getter device to room temperature.

9. A method according to claim 8, characterized in that:
A. said particulate non-evaporable getter material is chosen from the group consisting of titanium, zirconium and their hydrides; and
B. said particulate antisintering material is chosen from the group consisting of:
a) an alloy of zirconium with aluminium in which the weight percent of aluminium is 5-30%;
b) an alloy of zirconium with metals M₁ and M₂, wherein M₁ is chosen from the group consisting of vanadium and niobium and M₂ is chosen from the group consisting of iron and nickel; and
c) an alloy of Zr-V-Fe whose composition in weight percent, when plotted on a ternary composition diagram in weight percent Zr, weight percent V and weight percent Fe, lies within a polygon having as its corners the points defined by:
i) 75% Zr - 20% V - 5% Fe
ii) 45% Zr - 20% V -35% Fe
iii) 45% Zr - 50% V - 5% Fe

10. A method according to claim 9, characterized in that:
A. said ceramic support is alumina and said thin conductive film is a continuous film of aluminium having a thickness of between 0.1 µm and 5 µm;
B. said thicker metal layer is a continuous nickel layer having a thickness of between 5 µm and 50 µm;
C. said particulate non-evaporable getter material is titanium hydride having a particle size of between 20-60 µm with an average size of 40 µm;
D. said particulate antisintering material is a Zr-V-Fe alloy having a weight percent composition of 70% Zr, 24.6% V, 5.4% Fe having a particle size of between 20-60 µm with an average particle size of 40 µm; wherein, the weight ratio C : D of the electrophoretically deposited layer is from 1 : 4 to 4 : 1; and by comprising the additional steps of:
I. rinsing the coated support with acetone; and then
II. drying the coated support; and then
III. maintaining the coated support at a pressure less than 10⁻⁵ Torr (10⁻³ Pa) at a temperature between 350°C and 450°C for a period of time sufficient to release substantially all hydrogen from the titanium hydride thereby yielding metallic titanium; and thereby producing a coated support;
with the subsequent sintering step being carried out at a temperature between 900°C and 1000°C.

## Patentansprüche

1. Poröse nicht verdampfbare Gettervorrichtung (102; 202) mit
I. einem keramischen Substrat (104; 204);
II. einer porösen gesinterten Gettermaterialschicht, die umfaßt:
A. ein partikelförmiges nicht verdampfbares Gettermaterial (112, 112'; 206, 206') und
B. ein partikelförmiges Antisintermaterial (114, 114'; 208, 208'),
dadurch gekennzeichnet, daß sie des weiteren umfaßt:
III. eine elektrisch leitende Zwischenschicht (108, 110), die zumindest teilweise in das keramische Substrat und die poröse gesinterte Gettermaterialschicht eindiffundiert ist (210; 212, 212').

2. Gettervorrichtung nach Anspruch 1, dadurch gekennzeichnet, daß das keramische Substrat (104; 204) Aluminiumoxid ist.

3. Gettervorrichtung nach Anspruch 1, dadurch gekennzeichnet, daß das partikelförmige nicht verdampfbare Gettermaterial (112, 112'; 206, 206') aus der Gruppe ausgewählt ist, die aus Titan, Zirkon und ihren Hydriden besteht.

4. Gettervorrichtung nach Anspruch 1, dadurch gekennzeichnet, daß das partikelförmige Sintermaterial (114, 114'; 208, 208') aus der Gruppe ausgewählt ist, die aus Graphit, hochschmelzenden Metallen und metallischen Getterlegierungen besteht.

5. Gettervorrichtung nach Anspruch 4, dadurch gekennzeichnet, daß das Antisintermaterial eine Legierung auf Zirkonbasis ist.

6. Poröse nicht verdampfbare Gettervorrichtung (102; 202) nach den Ansprüchen 2 bis 5, dadurch gekennzeichnet, daß die elektrisch leitende Zwischenschicht umfaßt:
A. einen Dünnfilm (108) aus Aluminium; und
B. eine dickere Schicht (110) aus Nickel, die zumindest teilweise in das Aluminiumsubstrat (104; 204) und die poröse gesinterte Gettermaterialschicht eindiffundiert ist.

7. Gettervorrichtung nach Anspruch 6, dadurch gekennzeichnet, daß die Legierung auf Zirkonbasis aus der Gruppe ausgewählt ist, die aus folgendem besteht:
A. einer Legierung aus Zirkon mit Aluminium, wobei der Gewichtsprozentanteil von Aluminium 5-30 % beträgt;
B. einer Legierung aus Zirkon mit den Metallen M₁ und M₂, wobei M₁ aus der Gruppe ausgewählt ist, die aus Vanadium und Niob besteht und M₂ aus der Gruppe ausgewählt ist, die Eisen und Nickel umfaßt; und
C. einer Legierung aus Zr-V-Fe, deren Zusammensetzung in Gew.%, wenn sie in einem ternären Zusammensetzungsdiagramm in Gew.% Zr, Gew.% V und Gew.% Fe eingetragen ist, innerhalb eines Polygons liegt, dessen Eckpunkte wie folgt definiert sind:
i) 75 % Zr - 20 % V - 5 % Fe,
ii) 45 % Zr - 20 % V - 35 % Fe,
iii) 45 % Zr - 50 % V - 5 % Fe.

8. Verfahren zum Herstellen einer porösen nicht verdampfbaren Gettervorrichtung, gekennzeichnet durch die folgenden Schritte:
I. Beschichten eines keramischen Substrates (104; 204) mit einem dünnen leitenden Film (108);
II. Elektroplattieren des dünnen leitenden Filmes (108) mit einer dickeren Metallschicht (110), um ein elektroplattiertes Substrat zu erzeugen;
III. elektrophoretisches Beschichten des elektroplattierten Substrates mit einem Gemisch aus:
A. einem partikelförmigen nicht verdampfbaren Gettermaterial (112, 112'; 206, 206'); und
B. einem partikelförmigen Antisintermaterial (114, 114'; 208, 208'), um ein beschichtetes Substrat herzustellen;
IV. Sintern des beschichteten Substrates bei Temperaturen über Raumtemperatur, um die poröse nicht verdampfbare Gettervorrichtung zu erzeugen, wobei die dickere elektroplattierte Metallschicht (110) in das keramische Substrat (104; 204) und das elektrophoretisch beschichtete Gemisch diffundiert; und dann
V. Abkühlen der Gettervorrichtung auf Raumtemperatur.

9. Verfahren nach Anspruch 8, dadurch gekennzeichnet, daß
A. das partikelförmige nicht verdampfbare Gettermaterial aus der Gruppe ausgewählt ist, die aus Titan, Zirkon und ihren Hydriden besteht; und
B. das partikelförmige Antisintermaterial aus der Gruppe ausgewählt ist, die aus den folgenden Komponenten besteht:
a) einer Legierung aus Zirkon mit Aluminium, wobei der Gewichtsprozentanteil von Aluminium 5 - 30 % beträgt;
b) einer Legierung aus Zirkon mit den Metallen M₁ und M₂, wobei M₁ aus der Gruppe ausgewählt ist, die aus Vanadium und Niob besteht, und M₂ aus der Gruppe ausgewählt ist, die aus Eisen und Nickel besteht; und
c) einer Legierung aus Zr-V-Fe, deren Zusammensetzung in Gewichtsprozent, wenn sie in einem ternären Zusammensetzungsdiagramm in Gew.% Zr, Gew.% V und Gew.% Fe eingetragen ist, innerhalb eines Polygons liegt, dessen Eckpunkte wie folgt definiert sind:
i) 75 % Zr - 20 % V - 5 % Fe,
ii) 45 % Zr - 20 % V - 35 % Fe,
iii) 45 % Zr - 50 % V - 5 % Fe.

10. Verfahren nach Anspruch 9, dadurch gekennzeichnet, daß
A. das keramische Substrat Aluminiumoxid und der dünne leitende Film ein kontinuierlicher Film aus Aluminium mit einer Dicke zwischen 0,1 µm und 5 µm ist;
B. die dickere Metallschicht eine kontinuierliche Nickelschicht mit einer Dicke zwischen 5 µm und 50 µm ist;
C. das partikelförmige nicht verdampfbare Gettermaterial Titanhydrid mit einer Partikelgröße zwischen 20 - 60 µm und einer durchschnittlichen Größe von 40 µm ist; und
D. das partikelförmige Antisintermaterial eine Zr-V-Fe-Legierung ist, die eine Zusammensetzung mit 70 Gew.% Zr, 24,6 Gew.% V, 5,4 Gew.% Fe und eine Partikelgröße zwischen 20 - 60 µm sowie eine durchschnittliche Partikelgröße von 40 µm aufweist, wobei das Gewichtsverhältnis C:D der elektrophoretisch abgeschiedenen Schicht 1:4 bis 4:1 beträgt;
wobei das Verfahren die folgenden zusätzlichen Schritte aufweist:
I. Spülen des beschichteten Substrates mit Aceton; und dann
II. Trocknen des beschichteten Substrates; und dann
III. Halten des beschichteten Substrates unter einem geringeren Druck als 10⁻⁵ Torr (10⁻³ Pa) bei einer Temperatur zwischen 350°C und 450°C über eine ausreichende Zeitdauer, um im wesentlichen den gesamten Wasserstoff vom Titanhydrid freizugeben und auf diese Weise metallisches Titan zu erhalten und ein beschichtetes Substrat zu erzeugen;
wobei der nachfolgende Sinterschritt bei einer Temperatur zwischen 900°C und 1000°C durchgeführt wird.

## Revendications

1. Dispositif getter non évaporable poreux (102 ; 202) comprenant :
I. un support en céramique (104 ; 204) ;
II. une couche de matériau getter fritté poreux comprenant :
A. une matière fixatrice de gaz non évaporable particulaire (112, 112' ; 206, 206') et
B. une matière d'antifrittage particulaire (114, 114' ; 208, 208'),
caractérisé en ce qu'il comprend de plus :
III. une couche intermédiaire conductrice de l'électricité (108, 110) au moins partiellement diffusée (210 ; 212, 212') dans le support en céramique et la couche de matériau getter fritté poreux.

2. Dispositif getter selon la revendication 1, caractérisé en ce que le support en céramique (104 ; 204) est l'alumine.

3. Dispositif getter selon la revendication 1, caractérisé en ce que le matériau getter non évaporable particulaire (112, 112' ; 206, 206') est choisi dans le groupe constitué du titane, du zirconium et de leurs hydrures.

4. Dispositif getter selon la revendication 1, caractérisé en ce que la matière d'antifrittage particulaire (114, 114' ; 208, 208') est choisie dans le groupe constitué du graphite, de métaux réfractaires et des alliages getter métalliques.

5. Dispositif getter selon la revendication 4, caractérisé en ce que la matière d'antifrittage est un alliage à base de zirconium.

6. Dispositif getter non évaporable poreux (102 ; 202) selon les revendications 2 à 5, caractérisé en ce que ladite couche intermédiaire conductrice de l'électricité comprend :
A. une pellicule mince (108) d'aluminium ; et
B. une couche plus épaisse (110) de nickel au moins partiellement diffusé à l'intérieur du support d'alumine (104 ; 204) et la couche de matériau getter fritté poreux.

7. Dispositif getter selon la revendication 6, caractérisé en ce que l'alliage à base de zirconium est choisi dans le groupe constitué de :
A. un alliage de zirconium avec l'aluminium dans lequel le pourcentage en poids d'aluminium est de 5 à 30 % ;
B. un alliage de zirconium avec des métaux M₁ et M₂ où M₁ est choisi dans le groupe constitué du vanadium et du niobium et M₂ est choisi dans le groupe comprenant le fer ou le nickel et
C. un alliage de Zr-V-Fe dont la composition en pourcentage pondéral, quand elle est tracée sur un diagramme de composition ternaire en pourcentage pondéral de Zr, en pourcentage pondéral de V et en pourcentage pondéral de Fe, s'étend à l'intérieur d'un polygone ayant pour sommets les points définis par :
i) 75% Zr - 20% V - 5% Fe
ii) 45% Zr - 20% V - 35% Fe
iii) 45% Zr - 50% V - 5% Fe

8. Procédé pour fabriquer un dispositif getter non évaporable poreux, caractérisé en ce qu'il comprend les opérations consistant :
I. à revêtir un support en céramique (104 ; 204) avec une pellicule conductrice mince (108) ;
II. à électroplaquer la pellicule conductrice mince (108) avec une couche de métal plus épaisse (110) pour produire un support électroplaqué ;
III. à revêtir électrophorétiquement le support électroplaqué avec un mélange de :
A. un matériau getter non évaporable particulaire (112, 112' ; 206, 206') ; et
B. une matière d'antifrittage particulaire (114, 114' ; 208, 208') pour produire un support revêtu ;
IV. à fritter le support revêtu à des températures supérieures à la température ambiante pour produire le dispositif getter non évaporable poreux ; tandis que la couche métallique plus épaisse électroplaquée (110) se diffuse dans le support en céramique (104 ; 204) et le mélange revêtu électrophorétiquement ; et ensuite
V. à refroidir ledit dispositif getter à la température ambiante.

9. Procédé selon la revendication 8, caractérisé en ce que :
A. ledit matériau getter non évaporable particulaire est choisie dans le groupe constitué du titane, du zirconium et de leurs hydrures ; et
B. ladite matière d'antifrittage particulaire est choisie dans le groupe constitué de :
a) un alliage de zirconium et d'aluminium dans lequel le pourcentage en poids d'aluminium est 5 à 30 % ;
b) un alliage de zirconium avec des métaux M₁ et M₂ où M₁ est choisi dans le groupe constitué du vanadium et du niobium et M₂ est choisi dans le groupe constitué du fer et du nickel ; et
c) un alliage de Zr-V-Fe dont la composition en pourcentage pondéral, quand elle est tracée sur un diagramme de composition ternaire en pourcentage pondéral de Zr, en pourcentage pondéral de V et en pourcentage pondéral de Fe, s'étend à l'intérieur d'un polygone ayant pour sommets les points définis par :
i) 75% Zr - 20% V - 5% Fe
ii) 45% Zr - 20% V - 35% Fe
iii) 45% Zr - 50% V - 5% Fe

10. Procédé selon la revendication 9, caractérisé en ce que :
A. ledit support en céramique est de l'alumine et ladite pellicule conductrice mince est une pellicule continue d'aluminium ayant une épaisseur comprise entre 0,1 µm et 5 µm ;
B. ladite couche métallique plus épaisse est une couche continue de nickel ayant une épaisseur comprise entre 5 µm et 50 µm ;
C. ledit matériau getter non évaporable particulaire est l'hydrure de titane ayant une granulométrie comprise entre 20 et 60 µm avec une taille moyenne de 40 µm ;
D. ladite matière d'antifrittage particulaire est un alliage de Zr-V-Fe ayant une composition en pourcentage pondéral de 70 % de Zr, 24,6 % de V, 5,4 % de Fe ayant une granulométrie comprise entre 20 à 60 µm avec une granulométrie moyenne de 40 µm ; dans laquelle, le rapport pondéral C:D de la couche déposée électrophorétiquement est de 1:4 à 4:1 ; et - comprenant les étapes supplémentaires consistant :
I. à rincer le support revêtu avec de l'acétone ; et ensuite
II. à sécher le support revêtu ; et ensuite
III. à maintenir le support revêtu sous une pression inférieure à 10⁻⁵ Torr (10⁻³ Pa) à une température comprise entre 350°C et 450°C pendant une durée suffisante pour libérer pratiquement tout l'hydrogène de l'hydrure de titane, produisant ainsi du titane métallique ; et à produire ainsi un support revêtu ;
l'étape de frittage ultérieure étant effectuée à une température comprise entre 900°C et 1 000°C.
